

## UNITED STATES PATENT OFFICE

2,376,192

COLOR-FORMING COMPOUNDS HAVING  
SIX-MEMBERED RINGS

Ilmari F. Salminen, Paul W. Vittum, and Arnold Weissberger, Rochester, N. Y., assignors to Eastman Kodak Company, Rochester, N. Y., a corporation of New Jersey

No Drawing. Application January 12, 1943,  
Serial No. 472,166

10 Claims. (Cl. 95—88)

This invention relates to photographic color-forming compounds and particularly to color-forming compounds having six-membered rings.

The use of color-forming compounds which react with the development product of primary aromatic amino developing agent to form colored images on photographic development is well known and has been the subject of numerous prior patents. The dyes formed in this way are insoluble in water and in the ordinary photographic developing and fixing baths, although the silver images formed simultaneously with them during the photographic development may be removed from the photographic layer to leave pure dye images in the layer. The coupler compounds employed in this way may be added to the developing solution or in certain cases may be incorporated in the photographic layer prior to exposure. When the coupler compounds are incorporated in the developer solution, it is desired that they be sufficiently soluble in the developer solution so that amounts may be used which produce sufficiently high dye densities in the resulting photographic image. In many cases the coupler compounds are not sufficiently soluble in the developer and steps must be taken to increase their solubility, for example, by the introduction of a sulfonic group.

It is an object of the present invention to provide novel photographic coupler compounds having desirable color-forming properties. A further object is to provide coupler compounds which produce dyes of desirable light transmission characteristics for purposes of color photography. A still further object is to provide coupler compounds possessing sufficiently high activity toward the oxidized coupling developer that dyes of usable dye density may be produced.

These objects are accomplished by the use of certain coupler compounds having the following structural formulas:



A=hydrogen or phenyl

B=hydrogen, phenyl or acyl, e. g., acetyl

R=hydrogen or alkyl, e. g., methyl

R'=hydrogen.

The following examples illustrate the com-

pounds which we have found suitable for use according to our invention:

(1)

N-phenylimide of *b*-phenylaminogluconic acid

(2)

20 *b*-Acetylaminogluconic imide (tautomeric form of 2,6-dihydroxy-4-acetylaminopyridine)  
(Ber. 19, 2700)

(3)

30 *b*-Acetylamino-*a*-methyl glutamic imide (tautomeric form of 2,6-dihydroxy-4-acetylamino-3-methyl pyridine)  
(J. Chem. Soc. 88, 1750)

(4)



40 3-carbethoxy-2,6-diketo-4-imino piperidine (J. C. S. (1904) 85, 1756)

(5)



45

46

47

48

49

50

It will be noted that certain of the compounds which we have found suitable as coupler compounds having six-membered rings, are amino glutaconic imides. Compounds 1, 2 and 3 are substituted amino glutaconic imides. We have found that not all of the six-membered ring compounds having a structure similar to glutaconic acid are suitable for use as color couplers. For

example, the N-phenylimide of  $\beta$ -phenyl glutaconic acid and the N-phenyl imide of  $\beta$ -methyl glutaconic acid (Ann. 370, 78 and 71) couple very poorly and form photographic images which are not satisfactory in practice.

All of the compounds which we have found suitable for use as couplers have a methylene group between two carbon atoms, one of which is a carbonyl carbon atom. The methylene group is believed to be active in the color-forming reaction to couple with the developer oxidized with the development of the silver halide.

The following example illustrates a developing solution containing one of the coupler compounds used according to our invention:

## A

|                               |       |     |
|-------------------------------|-------|-----|
| p-Aminodimethylanilinesulfate | grams | 2.5 |
| Sodium sulphite anhydrous     | do    | 2   |
| Sodium carbonate anhydrous    | do    | 20  |
| Potassium bromide             | do    | 1   |
| Water to                      | liter | 1   |

## B

|                                                       |       |    |
|-------------------------------------------------------|-------|----|
| N-phenylimide of $\beta$ -phenylamine-glutaconic acid | grams | 2  |
| Sodium hydroxide, 10% solution                        | cc    | 10 |

For use, B is added to A.

In the foregoing example, we have described adding the coupler compound to the developing solution itself. Although it will essentially be employed in this way, the coupler compound may also be incorporated in the photographic layer prior to exposure and the colored image formed by development of the layer in the primary aromatic amino developing solution A indicated above. Special dispersing agents may be used for incorporating the coupler compound in the emulsion and in certain cases the coupler may be absorbed or adsorbed to the sensitive salt or may be combined with the sensitive salt as a chemical combination. In the case of multi-layer film, in which color forming compounds may be incorporated in one or more of the layers, it may be necessary to take special precautions to prevent wandering of the coupler compound from the sensitive layer in which it is incorporated. For example, the compounds may be incorporated in an emulsion layer in the manner described in Mannes and Godowsky U. S. Patents 2,304,939 and 2,304,940, granted December 15, 1942.

The specific coupler compounds illustrated above produce various colors upon coupling with the oxidation product of a primary aromatic amino developing agent. The colors produced are as follows:

- Compound 1—purple to blue.
- Compound 2—blue to cyan.
- Compound 3—blue to cyan.
- Compound 4—blue to cyan.
- Compound 5—blue to cyan.

The aromatic amino developing agents used with the coupler compounds of our invention include the mono, di and tri-aminoaryl compounds and their derivatives formed by substitution in the amino group as well as in the ring, such as alkyl-phenylenediamines and alkyltolylenediamines. These compounds are usually used in the salt form, such as the hydrochloride or the sulphate, which are more stable than the amines themselves. Suitable compounds are diethyl-p-phenylenediamine hydrochloride, monomethyl-p-phenylenediamine hydrochloride, dimethyl-p-phenyl-

enediamine hydrochloride and dimethyl-p-phenylenediaminesulphate. The p-aminophenols and their substitution products may also be used where the amino group is unsubstituted. All of these compounds have an unsubstituted amino group which enables the oxidation products of the developer to couple with the color-forming compounds to form a dye image.

Our development process may be employed for the production of colored photographic images in layers of gelatin or other carrier, such as collodion, organic esters of cellulose, or synthetic resins. The carrier may be supported by a transparent medium such as glass, a cellulose ester or a non-transparent reflecting medium such as paper or an opaque cellulose ester. The emulsion may be coated as a single layer on the support or as superposed layers on one or both sides of the support. The superposed layers may be differentially sensitized and the dyes formed therein by coupling may be bleached by an oxidizing agent such as chromic acid to colorless soluble compounds. The destruction of the dye in this way does not destroy the silver image and a silver image may be developed, bleached and developed to color a number of times, thus permitting the formation of natural color images in superposed layers as described, for example, in Mannes and Godowsky U. S. Patent No. 2,113,329.

30 The examples and compounds set forth in the present specification are illustrative only and it is to be understood that our invention is to be taken as limited only by the scope of the appended claims.

35 We claim:

1. A color-forming photographic developer comprising a primary aromatic amino developing agent and a coupler compound having the following formula:



50 where A is selected from the group consisting of hydrogen and phenyl radicals, B is selected from the group consisting of hydrogen, phenyl and acyl radicals, R is selected from the group consisting of hydrogen and alkyl and R' is hydrogen.

55 2. A color-forming photographic developer comprising a primary aromatic amino developing agent and a coupler compound comprising a  $\beta$ -amino glutaconic imide.

3. A color-forming photographic developer comprising a primary aromatic amino developing agent and a coupler compound comprising a  $\beta$ -acetyl amino glutaconic imide.

60 4. A color-forming photographic developer comprising a primary aromatic amino developing agent and a coupler compound comprising  $\beta$ -acetylaminoglutaconic imide.

5. A color-forming photographic developer comprising a primary aromatic amino developing agent and a coupler compound comprising glutazine.

65 6. The method of producing a colored photographic image in a gelatino-silver-halide emulsion layer, which comprises exposing the layer and developing it with a primary aromatic amino

developing agent in the presence of a coupler compound having one of the following formulas:



where A is selected from the group consisting of hydrogen and phenyl radicals, B is selected from the group consisting of hydrogen, phenyl and acyl radicals, R is selected from the group consisting of hydrogen and alkyl and R' is hydrogen.

7. The method of producing a color photographic image in a gelatino-silver-halide emulsion layer, which comprises exposing the layer and developing it with a primary aromatic amino developing agent in the presence of a coupler compound comprising a  $\beta$ -amino glutaconic imide.

8. The method of producing a color photo-

graphic image in a gelatino-silver-halide emulsion layer, which comprises exposing the layer and developing it with a primary aromatic amino developing agent in the presence of a coupler compound comprising a  $\beta$ -acetyl amino glutaconic imide.

9. The method of producing a color photographic image in a gelatino-silver-halide emulsion layer, which comprises exposing the layer and developing it with a primary aromatic amino developing agent in the presence of a coupler compound comprising  $\beta$ -acetyl amino glutaconic imide.

10. The method of producing a color photographic image in a gelatino-silver-halide emulsion layer, which comprises exposing the layer and developing it with a primary aromatic amino developing agent in the presence of a coupler compound comprising glutazine.

ILMARI F. SALMINEN.

PAUL W. VITTRUM.

ARNOLD WEISSBERGER.